# EUROPEAN PATENT SPECIFICATION

(11) **EP 3 486 349 B1**
(45) Date of publication and mention of the grant of the patent: **01.07.2020**
(21) Application number: 18212939.5
(22) Date of filing: 25.01.2011
(51) Int. Cl.: C23C 2/04, C22C 21/10, C23C 2/12, C22C 18/04, C23C 2/06, C23C 2/40, C23C 2/30

(54) **METAL-COATED STEEL STRIP**
METALLBESCHICHTETER STAHLSTREIFEN
BANDE D'ACIER REVÊTUE DE MÉTAL

(30) Priority: 25.01.2010 AU 2010900287
(43) Date of publication of application: 22.05.2019
(62) Divisional of application: 11734260.0
(73) Proprietor: Bluescope Steel Limited, Melbourne, Victoria 3000 (AU)
(72) Inventor: LOPEZ, Michael, Angel, New South Wales, 2530 (AU); RENSHAW, Wayne Andrew, New South Wales, 2526 (AU); MICALLEF, Andrew Vincent, Victoria, 3931 (AU); SETARGEW, Nega, New South Wales, 2525 (AU); DONALDSON, Paul, Victoria, 3930 (AU)
(74) Representative: Hedges, Martin Nicholas

(56) References cited:
- EP-A1- 1 225 246
- EP-A1- 1 466 994
- WO-A1-2009/111842
- CN-A- 101 457 320
- JP-A- 2009 256 703

## Description

The present invention relates to the production of strip, typically steel strip, which has a corrosion-resistant metal alloy coating that contains aluminium-zinc-silicon-magnesium as the main elements in the alloy, and is hereinafter referred to as an "Al-Zn-Si-Mg alloy" on this basis.

In particular, the present invention relates to a hot-dip metal coating method of forming an Al-Zn-Si-Mg alloy coating on a strip that includes dipping uncoated strip into a bath of molten Al-Zn-Si-Mg alloy and forming a coating of the alloy on the strip.

More particularly, the present invention is concerned with minimising the amount of top dross in the alloy coating bath. Top dross is undesirable from the viewpoints of cost of production and coating quality, as is discussed further below.

The Al-Zn-Si-Mg alloy of the present invention comprises the following ranges in % by weight of the elements Al, Zn, Si, and Mg:

| | |
|---|---|
| A1: | 45 to 60 % |
| Zn: | 35 to 50 % |
| Si: | 1.2 to 2.5% |
| Mg | 1.0 to 3.0% |

Depending on the end-use application, the metal-coated strip may be painted, for example with a polymeric paint, on one or both surfaces of the strip. In this regard, the metal-coated strip may be sold as an end product itself or may have a paint coating applied to one or both surfaces and be sold as a painted end product.

One corrosion resistant metal coating composition that is used widely in Australia and elsewhere for building products, particularly profiled wall and roofing sheets, is a 55%Al-Zn coating composition that also comprises Si. The profiled sheets are usually manufactured by cold forming painted, metal alloy coated strip. Typically, the profiled sheets are manufactured by roll-forming the painted strip.

The addition of Mg to this known composition of 55%Al-Zn-Si coating composition has been proposed in the patent literature for a number of years, see for example US patent 6,635,359 in the name of Nippon Steel Corporation, but Al-Zn-Si-Mg coatings on steel strip are not commercially available in Australia.

It has been established that when Mg is included in a 55%Al-Zn coating composition, Mg brings about certain beneficial effects on product performance, such as improved cut-edge protection.

The applicant has found that Mg-containing molten 55%Al-Zn coating metal is susceptible to increased levels of top dross generation compared to molten 55%Al-Zn coating metal that does not contain Mg.

The term "top dross" is herein understood to include any one or more of the following components on or near the surface of the molten bath:
(a) an oxide film on the surface of a molten bath,
(b) molten metal droplets covered by an oxide film,
(c) gas bubbles having an oxide film as the wall of the bubbles,
(d) intermetallic particles that are formed in the coating bath, including particles covered by an oxide film, and
(e) combinations of any two or more of gas, molten metal, and intermetallic particles covered by an oxide film.

Items (b), (c), (d), and (e) can be described as the result of entrainment of molten metal, gas, and intermetallic particles in the oxide film on or near the surface of the molten bath.

During a line trial to hot-dip metal coat a Mg-containing 55%Al-Zn alloy onto a steel strip that has been conducted by the applicant it was shown that the level of top dross generated in the coating bath was 6 to 8 times that of the top dross formed in a 55%Al-Zn alloy coating bath without Mg addition. Whilst not wishing to be bound by the following comment, the applicant attributes the generation of excessive top dross in Mg-containing molten coating alloys to the reactivity and rapid oxidation of Mg in the alloys and the changes in the properties of the liquid metal (for example, surface tension) that result from the addition of Mg to 55%Al-Zn alloy baths. More particularly, Mg has a higher affinity for oxygen compared with Al and therefore Mg oxidises much more readily than Al. This is evident from the standard free energy of formation (ΔG°) of the oxides which shows that: the thermodynamic driving force for oxide formation is much greater for Mg than for A1 (ΔG°_{Al2o3}=-934kJ/mol and ΔG°_{Mgo}=-1015kJ/mol at a bath operating temperature of 600°C). Moreover, turbulence in the melt surface enhances both the oxidation of molten metal in the bath and the entrainment of the oxide film in the coating bath. The entrainment of the oxide film in the coating bath results in the entrainment of molten metal, gas, and intermetallic particles in the oxide film in the molten bath and the consequential formation of the dross components described in items (b), (c), (d), and (e) above. This top dross has high volume fractions of voids, oxide stringers and dross intermetallic particles entrained in the top dross.

The amount of top dross generated has a significant impact on the cost of production of Mg-containing 55%Al-Zn alloy coated steel. Top dross must be removed from the bath surface periodically to prevent surface defects on the coated steel strip. The removal of top dross represents a cost to the producer of coated steel strip due to the cost of the removal process and the cost of top dross disposal or recycling. Reducing top dross generation provides an opportunity to significantly reduce the cost of production.

In addition, reducing top dross also provides an opportunity to lead to improved surface quality of the coated strip by reducing entrainment of oxide stringers and suspended dross particles.

The above discussion is not to be taken as an admission of the common general knowledge in Australia and elsewhere.

EP 1466994 discloses a plated steel sheet capable of securing excellent post-painting corrosion resistance and brightness, and the present invention makes it possible to produce a plated steel sheet excellent in post-painting corrosion resistance and paint coat image clarity by further adding one or more elements selected from among 0.01 to 0.5% of Ca, 0.01 to 0.2% of Be, 0.0001 to 0.2% of Ti, 0.1 to 10% of Cu, 0.001 to 0.2% of Ni, 0.01 to 0.3% of Co, 0.0001 to 0.2% of Cr and 0.01 to 0.5% of Mn, in mass, to the plated layer of the plated steel sheet. The center line average roughness Ra of the Zn alloy plated steel sheet is 1.0 mu m or less and the filtered waviness curve WCA thereof is 0.8 mu m or less, the Zn alloy plated steel sheet having on the surface thereof the plated layer containing 1 to 10% of Mg, 2 to 19% of A1 and 0.001 to 2% of Si in mass and other elements the total amount of which is suppressed to 0.5% or less in mass, with the balance consisting of Zn.

Other prior art methods are disclosed in EP 1225246, JP 2009/256703 and CN 101 457 320

The applicant has been able to reduce the top dross levels in molten Al-Zn-Si-Mg alloy baths by the addition to molten baths of Ca and Sr and the reduction in top dross levels has lead to benefits in terms of production costs and product quality. The addition of these elements is hereinafter referred to as the addition of "Ca and Sr". It is noted that the above reference to the addition of Ca and Sr is not intended to indicate that Ca is added before Sr. The present invention extends to situations in which Ca and Sr are added at the same time or at different times to molten baths.

The applicant found that this reduction in top dross generation in molten Al-Zn-Si-Mg alloy baths by the addition of Ca and Sr to the baths is due to changes in the entrainment of gas, molten metal and intermetallic particles in oxide films in top dross in the baths resulting from (a) changes to the apparent surface tension at the liquid metal/oxide interface as a result of the Ca and Sr addition and (b) changes in the nature of the oxide film as a result of the Ca and Sr addition. The changes in the nature of the oxide film reduce the level of oxide stringers formed, which in turn assists in an overall reduction in liquid droplet entrainment.

According to the present invention there is provided a method of forming an Al-Zn-Si-Mg alloy coating on a strip according to claim 1.

The method may include controlling the conditions in the molten bath to minimise entrainment of any one or more of molten metal, gas, and intermetallic particles in oxide films in the top dross layer.

Hence, the method may include controlling the composition of the bath to minimise the top dross layer in the molten bath, for example by minimising liquid droplet entrainment in oxide films in the top dross layer in the bath.
It is noted that all references to ppm in the specification are references to ppm by weights.

It is noted that the reference to amounts of elements such as Ca and Sr as part of the composition of a molten bath are understood herein to be references to the concentrations of the elements in the molten metal layer of the bath as opposed to the top dross layer in the bath. The reason for this is that it is the standard practice of the applicant to measure bath concentrations in the molten metal layers of molten baths.

It is also noted that the applicant found that Ca and Sr tend to segregate to the top dross layer of molten baths and, as a consequence the top dross layer becomes enriched with respect to Ca and Sr when compared to the metal layer. Specifically, if there is "x" wt.% of Ca or Sr in the molten metal layer of a molten bath, there will be a higher concentration of the element in the top dross layer of the bath. For example, the applicant found in laboratory work that in a bath with a nominal bath composition of 90 ppm Ca, the Ca content of the top dross layer increased to 100 ppm Ca. Similarly, the applicant found that in a bath with a nominal composition of 400 ppm Ca, the top dross layer was enriched substantially to 600 ppm. Similar enrichments were also observed for Sr in laboratory work. For example, in a bath with a nominal composition of 500 ppm Sr, after 3 hrs of processing the top dross layer was enriched in Sr to 700 ppm. And in a bath with a nominal composition of 750 ppm Sr, after 3 hrs of processing the top dross layer was enriched to 1100 ppm Sr. In practice, this means that, if it is required that there be "x" wt.% of Ca or Sr in the molten metal layer of a molten bath, it will be necessary to add an amount of Ca or Sr that is greater than "x" wt.% in the total bath to compensate for the higher concentration of Ca or Sr that will segregate to the top dross layer.

The composition of the bath may include more than 150 ppm Ca.

The composition of the bath may include more than 200 ppm Ca.

The composition of the bath may include less than 750 ppm Ca.

The composition of the bath may include less than 500 ppm Ca.

The Ca may be added to the bath as required. It could be by way of specific additions of Ca compounds on a continuous or a periodic basis. It could also be by way of the inclusion of Ca in A1 and/or Zn ingots that are provided as feed materials for the bath.

The composition of the bath may include more than 100 ppm Sr.

The composition of the bath may include more than 150 ppm Sr.

The composition of the bath may include more than 200 ppm Sr.

The composition of the bath may include less than 1250 ppm Sr.

The composition of the bath may include less than 1000 ppm Sr.

The Sr may be added to the bath as required. It could be by way of specific additions of Sr compounds on a continuous or a periodic basis. It could also be by way of the inclusion of Sr in A1 and/or Zn ingots that are provided as feed materials for the bath.

The amounts of Ca and Sr in the composition may be as described above, with adjustments to the amounts of each element to compensate for the effect of an addition of the other element on the top dross layer.

The method may include controlling the composition of the bath to minimise the top dross layer in the molten bath by including rare earth elements such as yttrium and a combination of rare earths and Ca and Sr in the composition of the bath.

The method may include controlling the composition of the bath to minimise the top dross layer in the bath by periodically monitoring the concentration of any one or more of Ca, Sr, and rare earth elements that are in the bath, and adding Ca, Sr, and rare earth elements as required to maintain the bath composition for the element or elements.

In a situation in which the Ca, Sr, and rare earth elements are part of ingots of other elements that are in the composition in the bath, the method may include selecting any one or more of the sizes of the ingots, the timing of the addition of the ingots, and the sequence of the addition of the ingots to maintain the concentration of Ca, Sr, and rare earth elements substantially constant or within a preferred range of + or - 10% for the elements.

The Al-Zn-Si-Mg alloy may comprise more than 1.0 % by weight Mg.

The Al-Zn-Si-Mg alloy may comprise more than 1.3 % by weight Mg.

The Al-Zn-Si-Mg alloy may comprise more than 1.5 % by weight Mg.

The Al-Zn-Si-Mg alloy may comprise less than 3 % by weight Mg.

The Al-Zn-Si-Mg alloy may comprise more than 2.5 % by weight Mg.

The Al-Zn-Si-Mg alloy may comprise more than 1.2 % by weight Si.

The present invention is described further by way of example with reference to the accompanying drawings of which:
Figure 1 is a schematic drawing of one embodiment of a continuous production line for producing steel strip coated with an Al-Zn-Si-Mg alloy in accordance with the method of the present invention;
Figure 2 is a graph of the mass of dross versus time for molten Al-Zn-Si alloy baths with and without Mg and with and without Ca in experiments on dross generation carried out by the applicant;
Figure 3 is a graph of the mass of dross versus time for molten Al-Zn-Si alloy baths with and without Mg and with and without Sr in experiments on dross generation carried out by the applicant;
Figure 4 presents selected results from the experimental work summarised in Figures 2 and 3 that highlights the impact of Ca and Sr on top dross generation;
Figure 5 is a graph of the mass of dross versus Ca content in Al-Zn-Si-Mg alloy baths after process times of 1 and 3 hours; and
Figure 6 is a graph of the mass of dross generated versus time during the course of a line trial carried out by the applicant.

With reference to Figure 1, in use, coils of cold rolled steel strip are uncoiled at an uncoiling station 1 and successive uncoiled lengths of strip are welded end to end by a welder 2 and form a continuous length of strip.

The strip is then passed successively through an accumulator 3, a strip cleaning section 4 and a furnace assembly 5. The furnace assembly 5 includes a preheater, a preheat reducing furnace, and a reducing furnace.

The strip is heat treated in the furnace assembly 5 by careful control of process variables including:(i) the temperature profile in the furnaces, (ii) the reducing gas concentration in the furnaces, (iii) the gas flow rate through the furnaces, and (iv) strip residence time in the furnaces (i.e. line speed).

The process variables in the furnace assembly 5 are controlled so that there is removal of iron oxide residues from the surface of the strip and removal of residual oils and iron fines from the surface of the strip.

The heat treated strip is then passed via an outlet snout downwardly into and through a molten bath containing an Al-Zn-Si-Mg alloy held in a coating pot 6 and is coated with Al-Zn-Si-Mg alloy. The Al-Zn-Si-Mg alloy is maintained molten in the coating pot by use of heating inductors (not shown). Within the bath the strip passes around a sink roll and is taken upwardly out of the bath. Both surfaces of the strip are coated with the Al-Zn-Si-Mg alloy as it passes through the bath.

After leaving the coating bath 6 the strip passes vertically through a gas wiping station (not shown) at which its coated surfaces are subjected to jets of wiping gas to control the thickness of the coating.

The coated strip is then passed through a cooling section 7 and subjected to forced cooling.

The cooled, coated strip is then passed through a rolling section 8 that conditions the surface of the coated strip.

The coated strip is thereafter coiled at a coiling station 10.

As is indicated above, the applicant has found that Al-Zn-Si-Mg alloy coating baths generate substantially greater amounts of top dross in the baths than is the case with conventional 55%Al-Zn alloy baths in the coating lines of the applicant.

As discussed above, the applicant has conducted a number of laboratory experiments and line trials to determine whether it is possible to reduce the amount of dross generated in an Al-Zn-Si-Mg alloy bath. As discussed above, the applicant found that it was possible to significantly reduce the level of top dross by the addition of Ca or Sr to Al-Zn-Si-Mg alloys in coating baths.

The experimental results on the effect of Ca and Sr additions to coating baths on the level of top dross generation in Al-Zn-Si-Mg alloy coating baths are summarized in Figures 2 to 5.

The experimental work was carried out on the following alloy compositions, in wt. % for (a) an Al-Zn alloy (referred to as "AZ" in the Figures) and (b) an Al-Zn-Mg alloy (referred to as "MAZ" in the Figures) and (c) these AZ and MAZ alloys plus parts per million (ppm) Ca and Sr additions to these compositions:
AZ: 55Al-43Zn-1.5Si-0.5Fe
MAZ: 53Al-43Zn-2Mg-1.5Si-0.5Fe
MAZ + 236 ppm Ca.
MAZ + 90 ppm Ca.
MAZ + 400 ppm Ca.
MAZ + 500 ppm Sr.
MAZ + 750 ppm Sr.
MAZ + 800 ppm Sr.

It is noted that the concentrations of Ca and Sr are the concentrations of these elements in the metallic parts of molten baths.

In the experimental work the top dross generation was simulated using a laboratory melting furnace and an overhead mechanical stirrer. The laboratory set-up consisted of the following components:
- A melting furnace with clay graphite crucible.
- A variable speed overhead mechanical stirrer with a support stand.
- Dross collector cup machined from high density sintered boron-nitride ceramic and having a series of drainage holes in the bottom of the cup and a series of upstanding handles to allow the cup to be positioned and removed from the crucible.
- Stainless steel impellor shaft.
- Impellor machined from high density sintered boron nitride ceramic.

The dross collector cup and the impellor were fabricated from a high temperature material that is non-wetting to molten AZ and MAZ alloys. The sintered boron nitride ceramic of these components provided excellent non-wetting characteristics and high temperature stability in the coating bath.

For each experiment, 15kg of the coating alloy of a required composition was formed in the crucible and held at the process temperature of 600°C. The dross collector cup was then inserted into the molten bath and was retained in the bath until the melt temperature reached the process temperature. Then the shaft impellor assembly was lowered into the bath until the impellor just touched the surface of the melt. The stirrer motor was then switched on and the stirring speed was adjusted to 60RPM. This experimental set-up resulted in shearing of the surface of the bath without creating a vortex so that at each revolution of the impellor a fresh melt was continuously exposed to air to generate dross. The dross generated was pushed to the side of the crucible and accumulated on the side of the crucible. At the end of each experiment the accumulated dross was removed from the crucible by lifting the dross collector cup from the crucible and allowing excess entrained bath metal to drain into the crucible via holes in the dross collector cup. What was left in the dross collector cup comprised the entrained bath metal and dross intermetallic particles covered with oxide film. This retained material was the top dross generated in each experiment.

The experiments were conducted for durations of 0.5, 1.2, and 3 hrs.

After each experiment the dross collected was removed and weighed and the results are plotted as shown in Figures 2 to 5.

Figures 2 to 4 are graphs of the mass of dross versus time for the molten alloy baths, with the Figure 2 results focusing on the results for the Ca alloys and the Figure 3 results focusing on the results for the Sr alloys and the Figure 4 results highlighting selected results for Ca and Sr from Figures 2 and 3.

Figure 5 is a graph of the mass of dross versus Ca content in molten alloy baths after process times of 1 and 3 hours.

Figures 2 to 5 clearly show that the level of top dross generated in an Al-Zn-Si-Mg alloy bath can be significantly reduced by additions of Ca or Sr to MAZ alloy coating baths. More particularly, Figures 2 to 5 show that:
(a) MAZ alloy coating baths generate significantly higher amounts of top dross that AZ alloy coating baths, and
(b) the amount of top dross decreases significantly with increasing amounts of Ca and Sr in the MAZ alloys.

The results shown in Figures 2 to 5 were further confirmed for Ca in a line trial conducted for approximately 2 weeks. The line trial was carried out on the above-mentioned AZ alloy to which Mg and Ca were added at different points in time during the course of the line trial. Figure 6 shows the dross collected during the line trial and that the results are consistent with what was observed in the laboratory work. In particular, Figure 6 shows that there was a substantial increase in the amount of dross generated in the molten bath with the addition of Mg to the bath and a substantial decrease in the amount of dross as a consequence of the addition of Ca to the bath.

As is indicated above, the applicant attributes the reduction in the dross level to reduction in the entrainment of molten metal, gas, and intermetallic particles in the oxide film in the molten bath (i.e. in the top dross layer in the bath) that resulted from (a) changes to the apparent surface tension at the liquid metal/oxide interface as a result of the Ca and Sr additions and (b) changes in the nature of the oxide film as a result of the Ca and Sr additions. The changes in the nature of the oxide film reduced the level of oxide stringers formed, which in turn assists in an overall reduction in liquid droplet entrainment. The changes in the entrainment lead to reductions in the level of top dross generation in molten Al-Zn-Si-Mg alloys.

Ca and Sr are examples of elements that can be added to a molten bath of an Al-Zn-Si-Mg alloy to reduce the entrainment of molten metal, gas, and intermetallic particles in the oxide film in the bath and thereby reduce the level of dross in the bath. Other bath additions include, by way of example, rare earth elements such as yttrium and combinations of rare earths and calcium and strontium and calcium/strontium.

In practice, the Ca and/or Sr may be added to the bath as required. It could be by way of specific additions of Ca and/or Sr compounds on a continuous or a periodic basis. It could also be by way of the inclusion of Ca and/or in A1 and/or Zn ingots that are provided as feed materials for the bath.

## Claims

1. A method of forming an Al-Zn-Si-Mg alloy coating on a strip, with the method including passing a steel strip via an outlet snout of a heat treatment furnace downwardly into and through a molten bath containing a molten Al-Zn-Si-Mg alloy layer and a top dross layer on the molten alloy layer with the molten alloy forming a coating of the molten alloy on the strip and removing the coated strip from the bath by passing the coated strip upwardly through the top dross layer external of the outlet snout, with the alloy comprising the following ranges in % by weight of the elements Al, Zn, Si, and Mg: Al: 45 to 60 %; Zn: 35 to 50 %; Si: 1.2 to 2.5%; and Mg: 1.0 to 3.0%; and with the method further including controlling the conditions in the molten bath to minimise the top dross layer in the molten bath by controlling the composition of the bath to minimise the top dross layer in the molten bath by controlling the composition of the bath to include (a) Ca in an amount that is more than 50 ppm Ca and less than 1000 ppm Ca, and (b) Sr in the bath.

2. The method defined in claim 1, including controlling the composition of the bath to include more than 150 ppm Ca.

3. The method defined in any of the preceding claims, including controlling the composition of the bath to include less than 750 ppm Ca.

4. The method defined in claim 3, including controlling the composition of the bath to include less than 500 ppm Ca.

5. The method defined in any of the preceding claims including controlling the composition of the bath to include more than 100 ppm Sr.

6. The method defined in claim 5, including controlling the composition of the bath to include more than 150 ppm Sr.

7. The method defined in claim 6, including controlling the composition of the bath to include more than 200 ppm Sr.

8. The method defined in any of the preceding claims, including controlling the composition of the bath to include less than 1250 ppm Sr.

9. The method defined in claim 8, including controlling the composition of the bath to include less than 1000 ppm Sr.

10. The method defined in any of the preceding claims, including controlling the composition of the bath to minimise the top dross layer in the molten bath by including rare earth elements such as yttrium and combinations of rare earths in the composition of the bath.

11. The method defined in any of the preceding claims wherein the AI-Zn-Si-Mg alloy comprises more than 1.0 % by weight Mg.

12. The method defined in any of the preceding claims wherein the Al-Zn-Si-Mg alloy comprises less than 3 % by weight Mg.

13. The method defined in any of the preceding claims wherein the Al-Zn-Si-Mg alloy comprises more than 1.2 % by weight Si.

## Patentansprüche

1. Verfahren zum Bilden einer Al-Zn-Si-Mg-Legierungsbeschichtung auf einem Band, wobei das Verfahren das Führen eines Stahlbandes über eine Auslaufschnauze eines Wärmebehandlungsofens nach unten in und durch ein Schmelzbad beinhaltet, das eine geschmolzene Al-Zn-Si-Mg-Legierungsschicht und eine Oberschlackeschicht auf der geschmolzenen Legierungsschicht beinhaltet, wobei die geschmolzene Legierung eine Beschichtung aus der geschmolzenen Legierung auf dem Band bildet, und Entnehmen des beschichteten Bandes aus dem Bad durch Führen des beschichteten Bandes nach oben durch die Oberschlackeschicht außerhalb der Auslaufschnauze, wobei die Legierung die folgenden Bereiche der Elemente AI, Zn, Si und Mg in Gew.-% aufweist: AI: 45 bis 60 %; Zn: 35 bis 50 %; Si: 1,2 bis 2,5 % und Mg: 1,0 bis 3,0 %; und wobei das Verfahren ferner das Steuern der Bedingungen im Schmelzbad beinhaltet, um die Oberschlackenschicht im Schmelzbad durch Steuern der Zusammensetzung des Bades zu minimieren, um die Oberschlackenschicht im Schmelzbad durch Steuern der Zusammensetzung des Bades, um (a) Ca in einer Menge, die höher ist als 50 ppm Ca und geringer als 1000 ppm Ca, und (b) Sr im Bad zu beinhalten, zu minimieren.

2. Verfahren nach Anspruch 1, beinhaltend das Steuern der Zusammensetzung des Bades, um mehr als 150 ppm Ca zu beinhalten.

3. Verfahren nach einem der vorhergehenden Ansprüche, beinhaltend das Steuern der Zusammensetzung des Bades, um weniger als 750 ppm Ca zu beinhalten.

4. Verfahren nach Anspruch 3, beinhaltend das Steuern der Zusammensetzung des Bades, um weniger als 500 ppm Ca zu beinhalten.

5. Verfahren nach einem der vorhergehenden Ansprüche, beinhaltend das Steuern der Zusammensetzung des Bades, um mehr als 100 ppm Sr zu beinhalten.

6. Verfahren nach Anspruch 5, beinhaltend das Steuern der Zusammensetzung des Bades, um mehr als 150 ppm Sr zu beinhalten.

7. Verfahren nach Anspruch 6, beinhaltend das Steuern der Zusammensetzung des Bades, um mehr als 200 ppm Sr zu beinhalten.

8. Verfahren nach einem der vorhergehenden Ansprüche, beinhaltend das Steuern der Zusammensetzung des Bades, um weniger als 1250 ppm Sr zu beinhalten.

9. Verfahren nach Anspruch 8, beinhaltend das Steuern der Zusammensetzung des Bades, um weniger als 1000 ppm Sr zu beinhalten.

10. Verfahren nach einem der vorhergehenden Ansprüche, beinhaltend das Steuern der Zusammensetzung des Bades, um die Oberschlackeschicht in dem Schmelzbad durch Einschließen von Seltenerdelementen wie Yttrium und Kombinationen von seltenen Erden in der Zusammensetzung des Bades zu minimieren.

11. Verfahren nach einem der vorhergehenden Ansprüche, wobei die Al-Zn-Si-Mg-Legierung mehr als 1,0 Gew.-% Mg umfasst.

12. Verfahren nach einem der vorhergehenden Ansprüche, wobei die Al-Zn-Si-Mg-Legierung weniger als 3 Gew.-% Mg umfasst.

13. Verfahren nach einem der vorhergehenden Ansprüche, wobei die Al-Zn-Si-Mg-Legierung mehr als 1,2 Gew.-% Si umfasst.

## Revendications

1. Procédé de formation d'un revêtement d'alliage Al-Zn-Si-Mg sur une bande, le procédé comprenant le passage d'une bande d'acier via une busette de sortie d'un four de traitement thermique vers le bas dans et à travers un bain fondu contenant une couche d'alliage de Al-Zn-Si fondu et une couche d'écume supérieure sur la couche d'alliage fondu avec l'alliage fondu formant un revêtement de l'alliage fondu sur la bande et retirant la bande enduite du bain par le passage de la bande enduite vers le haut à travers la couche d'écume supérieure à l'extérieur de la busette de sortie, avec l'alliage comprenant les plages suivantes en % en poids des éléments AI, Zn, Si et M : IA : 45 à 60% ; Zn : 35 à 50% ; Si : 1,2 à 2,5% ; et Mg : 1,0 à 3,0% ; et avec le procédé comprenant en outre le contrôle des conditions dans le bain fondu, afin de minimiser la couche d'écume supérieure dans le bain fondu par le contrôle de la composition du bain afin de minimiser la couche d'écume supérieure dans le bain fondu par le contrôle de la composition du bain afin d'inclure (a) du Ca dans une quantité supérieure à 50 ppm de Ca et inférieure à 1000 ppm de Ca, et (b) du Sr dans le bain.

2. Procédé selon la revendication 1 comprenant le contrôle de la composition du bain pour inclure plus de 150 ppm de Ca.

3. Procédé selon l'une quelconque des revendications précédentes, comprenant le contrôle de la composition du bain pour inclure moins de 750 ppm de Ca.

4. Procédé selon la revendication 3, incluant le contrôle de la composition du bain pour inclure moins de 500 ppm de Ca.

5. Procédé selon l'une quelconque des revendications précédentes, comprenant le contrôle de la composition du bain pour inclure plus de 100 ppm de Sr.

6. Procédé selon la revendication 5 comprenant le contrôle de la composition du bain pour inclure plus de 150 ppm de Sr.

7. Procédé selon la revendication 6, comprenant le contrôle de la composition du bain pour inclure plus de 200 ppm de Sr.

8. Procédé selon l'une quelconque des revendications précédentes, comprenant le contrôle de la composition du bain pour inclure moins de 1250 ppm de Sr.

9. Procédé selon la revendication 8 comprenant le contrôle de la composition du bain pour inclure moins de 1000 ppm de Sr.

10. Procédé selon l'une quelconque des revendications précédentes, comprenant le contrôle de la composition du bain pour minimiser la couche d'écume supérieure dans le bain fondu par l'inclusion d'éléments de terres rares tels que l'yttrium et une combinaison de terres rares dans la composition du bain.

11. Procédé selon l'une quelconque des revendications précédentes, dans lequel l'alliage Al-Zn-Si-Mg comprend plus de 1,0% en poids de Mg.

12. Procédé selon l'une quelconque des revendications précédentes, dans lequel l'alliage Al-Zn-Si-Mg comprend moins de 3% en poids de Mg.

13. Procédé selon l'une quelconque des revendications précédentes, dans lequel l'alliage Al-Zn-Si-Mg comprend plus de 1,2% en poids de Si.
